

May 16, 1961

M. M. MORSE

2,984,565

PHOTOGRAPHIC PROCESS AND COMPOSITION

Filed March 18, 1960



FIG. 1



FIG. 2

INVENTOR.  
*Morse M. Morse*  
BY  
*Brown and Mikulka*  
*and*  
*Gerald Altman*  
ATTORNEYS

1

2,984,565

## PHOTOGRAPHIC PROCESS AND COMPOSITION

Meroe M. Morse, Boston, Mass., assignor to Polaroid Corporation, Cambridge, Mass., a corporation of Delaware

Filed Mar. 18, 1960, Ser. No. 16,100

7 Claims. (Cl. 96—29)

The present invention relates to photography and, more particularly, to the production of photographic prints by silver transfer.

Silver transfer techniques generally involve subjecting a silver halide latent image to developing and dissolving reagents in the presence of a silver-receptive environment where a visible silver print is formed. For example, a fluid, such as an alkaline aqueous solution of a silver halide developing agent and a silver solvent, is applied to a pair of strata, for example a photoexposed silver halide stratum and a silver-receptive stratum that are superposed. Thereafter, the strata are maintained in superposed relation for a predetermined processing period during which the reagents develop exposed silver halide to silver and react with unreacted silver halide to form a soluble silver complex that is reduced to silver in the print-receptive stratum to form a positive print. The present invention contemplates improving silver transfer techniques with the aid of an additive, initially disposed, for example, either in the fluid or on one of the sheets, that serves to enhance the character of the resulting print.

The primary object of the present invention is to enhance the blackness of a silver transfer print with the aid of cysteine, otherwise known as alpha-amino-beta-thiol-propionic acid.

Other objects of the invention will in part be obvious and will in part appear hereinafter.

The invention accordingly comprises the process involving the several steps and the relation and order of one or more of such steps with respect to each of the others and the composition possessing the features, properties and the relation of components which are exemplified in the following detailed disclosure, and the scope of the application of which will be indicated in the claims.

For a fuller understanding of the nature and objects of the invention, reference should be had to the following detailed description taken in connection with the accompanying drawing wherein:

Figure 1 is an exaggerated cross-sectional view of photographic materials undergoing a preferred process embodying the present invention; and

Fig. 2 is an exaggerated cross-sectional view of the print produced by the process of Fig. 1.

Generally, Fig. 1 shows a silver halide processing fluid 10 spread in a uniformly thin layer between the adjacent superposed surfaces of a silver halide photosensitive sheet 12 and a silver print-receptive sheet 14. Such spreading, for example, is accomplished by advancing the sheets, together with the fluid, between a pair of pressure-applying rollers. Preferably, the liquid is sufficiently viscous to be readily controlled as it is spread, in accordance with the teachings of U.S. Patent No. 2,543,181, issued to Edwin H. Land on February 27, 1951. In accordance

2

with the present invention, the processing fluid contains cysteine, represented by the formula:



in viscous alkaline solution with a silver halide developing agent such as hydroquinone, a silver halide solvent such as sodium thiosulfate and a thickener such as a water-soluble polymer or gum or an insoluble emulsifiable oil. The cysteine is present in a concentration effective to render the resulting silver transfer image substantially more neutral in tone, e.g., blue-black, as compared with the image which would be obtained in its absence. In a preferred embodiment, the cysteine is present in a concentration, by weight of said solution, of about 0.001 to 0.60%. The photosensitive sheet includes a gelatino silver halide stratum 16 on a suitable support 18 and the print-receptive sheet includes a silver-receptive stratum 20 on a suitable support 22. Within a predetermined period after solution 10 is spread, the reagents therein form a negative print in silver halide stratum 16 by reducing silver halide to silver and react with unreacted silver halide to form a silver complex which diffuses into the layer of processing fluid to silver-receptive stratum 20 where it is reduced to silver to form a positive print. The presence of the cysteine is responsible for a considerably more neutral tone in the resulting print than would exist in its absence.

### Example

In a specific example of the foregoing process: gelatino silver halide stratum 16 is a moderately high speed gelatino iodobromide emulsion 0.0001 to 0.0009 inch thick of the type sold by Eastman Kodak under the trade name "Verichrome"; silver-receptive stratum 20, 1 to 8 microns thick, contains a silver precipitating agent of the type described in Patents Nos. 2,698,237 and 2,698,245, which issued on December 28, 1954 in the name of Edwin H. Land; and the formulation of processing fluid 10 is as follows:

|                                | Grams  |
|--------------------------------|--------|
| Hydroquinone                   | 52.0   |
| Sodium thiosulfate             | 14.5   |
| Cysteine                       | 5.2    |
| Sodium hydroxide               | 54.6   |
| Sodium sulfite                 | 78.0   |
| Sodium carboxymethyl cellulose | 93.0   |
| Water                          | 1860.0 |

Here, silver halide stratum 16 and silver-receptive stratum 20 are maintained in superposed relation with processing fluid 10 therebetween for a period of approximately from 40 to 120 seconds in duration. At the end of this period, silver-receptive stratum 20 and layer of solution 10 are

stripped from silver halide stratum 16 to display a positive print of substantially richer and blacker tone than would have been obtained in the absence of cysteine. The presence of cysteine also appreciably increases the effective speed of the process.

The proportions of the ingredients of processing fluid 10 may be varied within wide limits. However, where the processing period is as specified, within the range of from 40 to 120 seconds in accordance with the now conventional duration of silver diffusion transfer processing periods, practical results are achieved where, by total weight of the fluid, the developing agent ranges from 1 to 8%, the silver halide solvent from 0.3 to 10%, and the thickener is in sufficient concentration to impart to the fluid a viscosity of from 100 to 200,000 centipoises at a temperature of 20° C. Practical results are achieved in the process of the above example when the cysteine

ranges, by total weight of the fluid, from 0.001 to 0.40% of the fluid.

The present invention may be applied to a variety of silver transfer processes other than the one specifically referred to above. The fluid may be spread either between the adjacent faces or on one of the remote faces of the superposed silver halide silver-receptive strata before or after photoexposure. The fluid itself may contain a silver precipitating agent in the presence of which print formation occurs, so that the solidified layer of said fluid contains the desired silver transfer image, in accordance with the principles of Patent No. 2,662,822 issued to Edwin H. Land on December 15, 1953, e.g., a composition like that of Example 1 of said patent. In fact, the additive of the present invention is especially useful in the processes of the latter patent to render more blue black the sepia images which are normally obtained from using the compositions of the aforesaid patent. When used in these compositions, the additive of the present invention is preferably present in proportions varying from 0.002 to 0.60% of the composition by weight. It may also be usefully employed in processes which provide a support with a photosensitive coating by application of a photosensitive material in accordance with the principles of United States Patent No. 2,846,309 granted August 5, 1958 to Edwin H. Land. Before photoexposure, such a process may initiate development to provide a dynamic photosensitive stratum in which a latent image later formed develops spontaneously in accordance with the principles of United States application Serial No. 498,672, filed April 1, 1955 in the name of Edwin H. Land. The two sheets may be stripped apart to uncover the resulting print or may be retained in superposed relation, when the maximum density of the negative is small compared to the maximum density of the positive print, in accordance with the teachings of United States Patent No. 2,861,885, granted November 25, 1958 to Edwin H. Land. When the various materials are associated in the form of a film unit having a pair of sheets and a container whose contents are to be spread between the sheets, the photographically active materials, including the cysteine, may be carried at a variety of locations, e.g., in the container or on one of the sheets. The photosensitive emulsion may be coated over the silver-receptive stratum, with the processing liquid being applied to the surface of the emulsion. After the desired transfer has been effected, the emulsion layer is stripped off.

The present invention thus is based upon the discovery of the unique properties of cysteine in relation to silver diffusion transfer processes and compositions useful therein.

This application is a continuation in part of my co-pending application, Serial No. 619,604, filed October 31, 1956 (now abandoned).

Since certain changes may be made in the above process

and composition without departing from the scope of the invention herein involved, it is intended that all matter contained in the above description or shown in the accompanying drawing shall be interpreted as illustrative and not in a limiting sense.

What is claimed is:

1. A photographic composition comprising an alkaline aqueous solution of a silver halide solvent fixer, a silver halide developing agent and cysteine, said cysteine ranging from about 0.001 to 0.60%, said developer ranging from about 1 to 8% and said silver halide solvent fixer ranging from about 0.3 to 10%, by total weight of said composition.

2. The photographic composition of claim 1, wherein said composition is a fluid possessing a viscosity of from 100 to 200,000 centipoises at a temperature of 20° C.

3. The photographic composition of claim 1, wherein said solution includes a silver precipitating agent.

4. A photographic process for producing a visible print, said process comprising the steps of applying a processing liquid to an exposed silver halide emulsion and effecting development of said exposed silver halide by a silver halide developing agent, reacting a silver halide solvent with at least a portion of the unexposed silver halide to form a soluble silver complex, and transferring said soluble silver complex to a silver-receptive stratum in superposed relationship with said silver halide emulsion, said silver-receptive stratum containing a silver precipitating agent whereby said transferred silver complex is precipitated to form said visible print, said process being effected in the presence of cysteine in a concentration, by total weight of said processing liquid, of about 0.001 to 0.60%.

5. The photographic process of claim 4, wherein said silver halide developing agent ranges from about 1 to 8%, and said silver halide solvent ranges from about 0.3 to 10%, by total weight of said liquid.

6. The photographic process of claim 5, wherein said liquid contains a thickener in sufficient quantity to impart a viscosity of from 100 to 200,000 centipoises at a temperature of 20° C.

7. The photographic process of claim 4, wherein said silver precipitating agent is contained in said processing liquid, and said visible print is contained in a solidified layer of said processing liquid.

#### References Cited in the file of this patent

#### UNITED STATES PATENTS

- |    |           |        |                |
|----|-----------|--------|----------------|
| 50 | 2,449,153 | Urbach | Sept. 14, 1948 |
|    | 2,740,715 | Land   | Apr. 3, 1956   |

#### OTHER REFERENCES

Chem. Abstracts, 41, 2016d (1947).

Chem. Abstracts, 33, 2498 (1939).